

## UNITED STATES PATENT OFFICE

IRVING R. VALENTINE, OF ERIE, PENNSYLVANIA, ASSIGNOR TO GENERAL ELECTRIC COMPANY, A CORPORATION OF NEW YORK

## TREATMENT OF MALLEABLE CASTINGS

No Drawing.

Application filed May 20, 1926. Serial No. 110,546.

My present invention relates to malleable cast iron, and more particularly to the heat treatment of malleable castings.

In my copending application, Serial No. 5 75,665, filed December 19, 1925, and of which the present application is a continuation in part, there is disclosed a method for treating malleable castings whereby embrittlement of the castings during the galvanizing 10 process is prevented. Such castings, however, in actual practice are frequently exposed to varying weather conditions and are, therefore, subjected to wide changes in temperature, and I have found that under certain 15 conditions, as where castings are subjected to temperatures well below 0° C., brittleness may sometimes occur after the castings have been galvanized, even though no brittleness developed during the galvanizing process 20 itself.

It is one of the objects of my invention to provide a method of treating malleable castings whereby such castings are rendered free from embrittlement not only during, but 25 subsequent to the galvanizing process.

It is a further object of my invention to provide means for restoring either black or galvanized malleable castings, which have become embrittled, to a normal or unembrittled 30 condition.

According to the present invention, I heat malleable castings to a temperature which is within the range of 100° C. and 540° C. and age the castings at this temperature for 35 a period of time varying from 3 to 72 hours, the ageing period and temperature employed varying according to the condition of the casting. Copper coated galvanized castings treated in this manner are rendered immune 40 from embrittlement when submitted to cold tests subsequent to the galvanizing process, while castings which have been rendered brittle either in the galvanizing process or by other means are restored to normal, un- 45 embrittled condition.

In carrying out my invention malleable castings are galvanized substantially in the manner described in my prior application above referred to. The malleable castings 50 are first cleaned by placing them in an acid

solution. Although a sand blast might be employed for this purpose, I have found that the latter method of cleaning iron is generally unsatisfactory since there is a tendency to leave a small thin film of sand on the metal which is detrimental to the process employed. After the iron has been removed from the acid solution, it is provided with a relatively thin copper coating which is obtained by dipping the iron momentarily in a copper sulphate 55 solution to which a mercury salt and concentrated sulphuric acid have been added, and which may advantageously be kept in an agitated condition by means of any suitable stirring device.

The proportions of materials employed in the solution are substantially as follows:

|                             |     |         |
|-----------------------------|-----|---------|
| Water                       | 1   | gallon. |
| Copper sulphate             | 2.5 | pounds. |
| Mercurous nitrate           | 1   | oz..    |
| Concentrated sulphuric acid | 1/2 | pound.  |

These figures represent approximate amounts only and may vary within certain limits both above and below the figures given. Although 75 the use of copper sulphate and mercurous nitrate gives very satisfactory results, other copper salts may be substituted for the sulphate if desired, and practically any mercury salt may be substituted for the mercurous 80 nitrate. While a relatively small amount of mercury salt will usually be employed, larger amounts may be used without causing any deleterious effect, since the mercury which adheres to the iron will be distilled in the 85 presence of the molten zinc.

For the successful galvanizing of malleable castings, according to the method disclosed in my prior application, it is necessary 90 that the copper form an adherent coating on the malleable iron. I have found that, by employing a mercury salt in the copper solution such a coating may be obtained; that the appearance of the copper deposit is thereby improved and that it cannot ordinarily be 95 rubbed off.

After the malleable iron is dipped in the copper sulphate solution, it is rinsed in water or alcohol and dried by heating to a temperature sufficiently high to drive off any mois- 100

ture. The casting is then immersed in a bath of molten zinc having a temperature of approximately 450° C. thereby providing the galvanized coating. As thus far described, 5 my invention is substantially the same as disclosed in my prior application, Serial No. 75,665.

After the castings have been galvanized, they are quenched in warm water having a 10 temperature of about 80° C., and are then transferred to a heated compartment where the castings are maintained or aged at a temperature between 120° C. and 145° C. for a period of approximately 6 hours, after which 15 the castings are removed and cooled in the air. Although I find a temperature range from 120° C. to 145° C. to be most suitable for carrying my invention into effect, this temperature range may be varied considerably.

20 In general, however, the temperature employed will not be lower than 100° C. nor higher than 165° C., since above the latter temperature the zinc coating has a tendency to peel. Likewise, although the most suitable 25 period for ageing will be found to be approximately 6 hours, this period may be considerably longer. Good results may furthermore be obtained by ageing the castings for as short a period as three hours, although in 30 the latter case, it will be found advisable to cool the castings quickly at the end of the ageing period, as by immersing in water, rather than to cool them in air. I have found from numerous tests that malleable iron 35 castings which have been galvanized and heat treated, as above described, are not only free from embrittlement during the galvanizing process, but that they will not subsequently become embrittled even when subjected to relatively low temperatures.

If desired, a similar heat treatment may be applied to malleable castings which have received no treatment, such as a copper coating, prior to galvanizing. In this case, however, 45 it will usually be found advisable to age the castings at an elevated temperature for a longer period of time than when the castings are copper coated, although otherwise the process is the same. For example, 50 ordinary malleable castings may be galvanized in the usual manner, by applying to the casting, molten zinc having a temperature of approximately 450° C. The castings are then quenched in warm water of approximately 55 80° C. and thereafter aged in a heated compartment, at a temperature which may range from 120° C. to 145° C., and for approximately 36 hours, after which the castings are removed and cooled in the air. Although 60 the average ageing period of 36 hours will be found satisfactory, this period may vary considerably, but usually will not be less than 6 hours or more than 72 hours in duration. Likewise, although 120° C. to 65 145° C. indicates the most desirable range of

temperature to be employed in the ageing process, this range may be extended both above and below the figures given. Usually the temperature employed will not be below 100° C. nor above 165° C., the latter temperature indicating the point above which a galvanized coating will peel.

If the heating of the galvanized casting is carried out in a furnace, care should be taken to protect the casting from free flames or from the action of the products of combustion. Although the application of molten zinc to malleable castings will ordinarily cause embrittlement of the castings, I have found that when the castings are submitted to the heat treatment indicated above, the galvanized castings are free from embrittlement, and the zinc coating is uninjured.

Malleable castings are frequently rendered extremely brittle from other causes than galvanizing, and I have found from numerous tests that this extreme brittleness may be removed by heating the castings to a temperature which, as a rule, will be in excess of that employed in connection with this heat treatment of galvanized castings, and by then ageing the castings for a period of time varying from 6 to 72 hours.

While it has previously been suggested that brittle malleable castings may be restored by heating to an elevated temperature such as 675° C. and then quenching, the apparatus employed in connection with such high temperature treatment is necessarily expensive and complicated, and it has been my experience that such heat treatment does not uniformly restore brittle castings to normal condition, due possibly to variation in the composition of the castings.

According to the present invention, malleable castings which have become embrittled are heated to a temperature of approximately 300° C., maintained or aged at this temperature for a period of approximately 36 hours and then cooled in air. While both the temperature and the ageing period given are indicative of the best mode of carrying my invention into effect they may vary to a considerable extent. In general, the temperature employed will not be less than 100° C. nor over 540° C. and the ageing period will range from 6 to 72 hours in duration, the lower ageing period being usually associated with the higher temperature and vice versa. Brittle castings treated in this manner are restored to normal condition and show uniformly a complete absence of brittleness, even after having been subjected to very low temperature tests. Of course, castings which have become brittle by galvanizing could be restored by heating to approximately 300° C. and ageing. This temperature, however, would destroy the zinc coating and necessitate further galvanizing.

Although I am at the present time not pre-

pared to give a theoretical explanation of the action that takes place in malleable castings when they are aged for prolonged periods at temperatures above 100° C. but below 540° C., 5 I have nevertheless demonstrated by a great number of tests that by such a treatment copper coated castings are rendered immune from subsequent embrittlement and that brittle malleable castings are restored to a normal unembrittled condition.

10 What I claim as new and desire to secure by Letters Patent of the United States is:

1. The method of treating zinc coated malleable cast iron which comprises ageing the 15 casting at a temperature above 100° C. but below a temperature at which the zinc coating will peel.

2. The method of treating zinc coated malleable cast iron which comprises ageing the 20 casting for at least three hours at a temperature within the range of 100° C. to 165° C.

3. The method of treating malleable cast iron which comprises applying a zinc coating at an elevated temperature to the casting, 25 quenching the casting, and ageing the casting at a temperature above 100° C. but lower than the temperature at which the zinc coating will peel.

4. The method of treating malleable cast 30 iron which comprises applying a copper coating to the casting, superimposing a zinc coating on the said copper coating, and ageing the casting at a temperature above 100° C. but lower than the temperature at which the zinc 35 coating will peel.

5. The method of treating malleable cast 40 iron which comprises providing the casting with a copper coating, applying molten zinc to the copper coating, quenching the casting, and ageing it at a temperature above 100° C. but not in excess of 165° C.

6. The method of treating malleable cast 45 iron which comprises applying a copper solution to the casting to provide a copper coating thereon, applying molten zinc to the copper coating, quenching the casting, ageing the casting at an elevated temperature not in excess of 165° C. and air cooling.

7. The method of treating malleable cast 50 iron which comprises applying to the casting a copper solution containing a mercury salt to provide a metal coating thereon, applying molten zinc to the coated casting, quenching the casting and ageing it at an elevated temperature not in excess of 165° C.

8. The method of treating malleable cast 55 iron which comprises applying a copper coating to the iron, applying molten zinc to said copper coating, quenching the casting and ageing it at a temperature within the range of 120° C. to 145° C. for approximately 6 hours.

9. The method of treating malleable cast 60 iron which comprises ageing the casting at a temperature higher than 100° C. but not

in excess of 540° C., and then cooling in air.

10. The method of treating malleable cast iron which comprises heating the casting to a temperature above 100° C. but not in excess of 540° C., and maintaining the casting at 70 said temperature for a period of at least six hours.

11. The method of treating malleable cast iron which comprises ageing the casting at a temperature of approximately 300° C. for 75 approximately 36 hours.

12. The method of treating malleable cast iron which comprises ageing the casting at a temperature of approximately 300° C.

13. The method of restoring a brittle malleable casting to normal condition which comprises ageing the casting at a temperature within the range of 100° C. to 540° C., and for a period of at least six hours.

14. The method of restoring a brittle malleable casting to normal condition which comprises ageing the casting at a temperature within the range of 100° C. to 540° C.

15. The method of treating zinc coated malleable cast iron which comprises ageing 90 the casting for a period of time varying from 3 to 72 hours and at a temperature within the range of 100° C. to 165° C.

16. The method of treating malleable cast iron which comprises ageing the casting for 95 a period of time varying from 3 to 72 hours and at a temperature within the range of 100° C. to 540° C.

In witness whereof, I have hereunto set my hand this 17th day of May, 1926.

IRVING R. VALENTINE.

105

110

115

120

125

130